

# United States Patent [19]

Brailowsky et al.

[11] 3,855,374

[45] Dec. 17, 1974

[54] **METHOD OF MAKING  
MAGNETICALLY-ANISOTROPIC  
PERMANENT MAGNETS**

[75] Inventors: **Vladimir Brailowsky, Birmingham;  
Erwin A. Alson, Fraser, both of  
Mich.**

[73] Assignee: **General Motors Corporation,  
Detroit, Mich.**

[22] Filed: **Dec. 22, 1972**

[21] Appl. No.: **317,785**

**Related U.S. Application Data**

[63] Continuation-in-part of Ser. No. 51,751, July 2, 1970, abandoned.

[52] **U.S. Cl.** ..... **264/24**, 252/62.58, 252/62.63,  
264/56.61, 264/86, 264/DIG. 58

[51] **Int. Cl.** ..... **C04b 35/26**

[58] **Field of Search** ..... 252/62.58, 62.63; 264/61,  
264/DIG. 58, 24, 86, 56

[56] **References Cited**

**UNITED STATES PATENTS**

2,762,777 9/1956 Went et al. ..... 252/62.63 X

|           |         |                |             |
|-----------|---------|----------------|-------------|
| 2,980,617 | 4/1961  | Ireland .....  | 252/62.63 X |
| 3,113,927 | 12/1963 | Cochardt ..... | 252/62.63 X |
| 3,424,685 | 1/1969  | Pierrot .....  | 252/62.63 X |

**FOREIGN PATENTS OR APPLICATIONS**

|           |        |                     |           |
|-----------|--------|---------------------|-----------|
| 1,471,405 | 9/1969 | Germany .....       | 252/62.63 |
| 754,626   | 8/1956 | Great Britain ..... | 252/62.63 |

*Primary Examiner*—Robert F. White

*Assistant Examiner*—Thomas P. Pavelko

*Attorney, Agent, or Firm*—George A. Grove

[57]

**ABSTRACT**

A method of making a permanent magnet of the hard ferrite type having a formula  $[\text{SrO}_0.6 \text{Fe}_2\text{O}_3]$   $\text{SrO}_0.6 \text{Fe}_2\text{O}_3$  is disclosed. The process comprises the critical step of adding a compound selected from the group consisting of boric acid and boric oxide to magnetite and a source of SrO during the mixing [a] and milling step prior to calcining of the mixture. Superior magnets are produced over those achieved by the process where the boric acid or boric oxide is introduced after calcining of magnetite and a source of SrO.

**5 Claims, 3 Drawing Figures**



PATENTED DEC 17 1974

3,855,374



Fig. 1



Fig. 2



Fig. 3

**METHOD OF MAKING  
MAGNETICALLY-ANISOTROPIC PERMANENT  
MAGNETS**

This application is a Continuation-In-Part of Ser. No. 51,751, filed July 2, 1970, now abandoned.

This invention relates to hard ferrite magnets and, more particularly, to a method of making magnetically-anisotropic permanent magnets of the hard ferrite type having improved magnetic properties.

The term "hard" ferrites, as used herein, refers generally to ferrite having a hexagonal crystalline lattice of the structure of the mineral magnetoplumbite and a formula  $\text{SrO} \cdot 6\text{Fe}_2\text{O}_3$ . The term "permanent" magnets, as used herein, refers to those magnets formed of hard magnetic materials in which, once magnetized, the magnetization is retained in the absence of a magnetizing field and they themselves serve to supply an external field.

The current widespread use of the permanent magnets is due, in general, to their desirable magnetic properties and their relatively low cost. Of the magnetic properties desired in permanent magnets one of the most important is a high coercive force. A high coercive force is needed to assure the magnetic stability in the presence of relatively high demagnetizing fields. This is an important consideration for dc motor applications, an important use of permanent magnets today, where demagnetizing fields can be high. Two other magnetic properties of importance in permanent magnet applications are residual flux density or remanence which remains when the "saturating" magnetizing force is reduced to zero and maximum magnetic energy product which is a measure of the maximum magnetic energy the given magnet can develop in its magnetic gap. Materials having the highest possible energy product, remanence and coercive force are used as permanent magnets.

Since the introduction of hard ferrite type permanent magnets, the ferrite technology has been directed to increasing the maximum energy, remanence and coercive force. The first major advance in this field came with the discovery that the maximum energy could be increased about threefold by orienting the ferrite particles along a preferred magnetic axis using a magnetic field. The orientation is accomplished by dispersing the hard ferrite particles in a slurry or other mobile state and then pressing the material into a body while under the influence of a directional magnetic field to align the ferrite particles whereby their easy direction of magnetization is more or less parallel to the applied field. Following orientation, the pressed body is sintered to produce the finished magnet which is then magnetized in the direction of orientation.

Since this discovery, efforts to increase the magnetic properties of oriented ferrite magnets have proceeded in two directions. The first is to increase magnetic properties by increasing the purity of the ferric oxide ( $\text{Fe}_2\text{O}_3$ ) used in producing the ferrite. Since ferric oxide is the principal ingredient of the starting composition, it was thought that by increasing the purity of  $\text{Fe}_2\text{O}_3$  improved properties would result. This technique has resulted in an improvement of the properties, but has also resulted in increasing the cost of fabricating ferrite magnets. The second approach is to increase maximum energy product and remanence by raising the sintering temperature of the oriented magnet to the range  $2,250^\circ$  to  $2,400^\circ$  F. However, past experience has

shown that the increase in the remanence on raising of the sintering temperature is accompanied by a decrease in coercive force. The first effect is apparently due to an increase in apparent density of the body while the

5 second effect appears to be a result of grain growth. Various additives such as silica, alumina, titania, or boric acid have been added to the ferrite prior to sintering to inhibit grain growth accompanying sintering with some beneficial effects. For example, commercial per-

10 manent magnets made with such an additive and sintered in the range of  $2250^\circ$  to  $2400^\circ$  F have a remanence,  $B_r$ , generally in excess of 3500 gauss and a maximum energy product,  $(\text{BH})_{max}$ , approaching  $3.5 \times 10^6$  gauss-oersteds. However, the coercive force  $H_c$  is found to decrease usually falling below 2000 oersteds which is undesirable in certain commercial applications where strong demagnetizing fields are present. For many such applications, it is desirable to have not only the remanence greater than 3500 gauss and the maximum energy product greater than  $3.0 \times 10^6$  gauss-oersteds, but also the coercive force in excess of 3000 oersteds. In addition, the magnets should be relatively inexpensive to produce.

20 Accordingly, it is among the principal objects of our invention to provide an inexpensive magnetically-anisotropic permanent magnet having improved magnetic properties and a method of making the same using magnetite ore instead of ferric oxide.

25 It is another object of our invention to provide a method of making improved hard ferrite compositions for use in making permanent magnets wherein relatively high magnetic properties are obtainable at relatively low sintering temperatures.

30 It is a further object of our invention to provide a method of making magnetically-anisotropic permanent magnets of the hard ferrite type using relatively inexpensive, raw grade magnetite ore, having a maximum energy product in excess of  $3.0 \times 10^6$  gauss-oersteds, a remanence in excess of 3500 gauss and a coercive force in excess of 3000 oersteds.

35 These and other objects are accomplished, in the preferred embodiment of our invention, by an improved ferrite manufacturing process including the steps of mixing magnetite ( $\text{Fe}_3\text{O}_4$ ) and strontium carbonate with a minor addition of boric acid in water, milling the compounds to form a homogeneous mixture thereof, drying the homogeneous oxide mixture, screening the resulting cake, tumbling the mixture to form a free-flowing powder, and then calcining the mixture at about  $2100^\circ$  F to form a ferrite. The calcined ferrite is then comminuted in water to a particle size which is 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665

form the hard ferrite composition which is then formed into a magnetically-anisotropic magnet.

Other objects and advantages of our invention will become apparent from the following detailed description of the invention, reference being had to the accompanying drawings of which:

FIG. 1 is a flow diagram of our improved process for making permanent magnets;

FIG. 2 is a graph showing the variation in remanence, coercive force and density with sintering temperatures of ferrite magnets made in accordance with our improved process; and

FIG. 3 is a graph showing the demagnetization portion of the hysteresis loop for two samples made by our improved process and subjected to different soak times at a sintering temperature of 2100° F.

In our improved method for fabricating hard, magnetically-anisotropic permanent magnets of the hard ferrite type, the proportions of raw materials are first weighed out as shown in FIG. 1, block 10. In accordance with the principal feature of our invention, the raw materials include predominately magnetite ( $Fe_3O_4$ ) with a source of the bivalent metal oxide,  $SrO$ , such as the oxides or carbonates of strontium, and a minor addition of a source of boron such as boric acid or boric oxide. In our preferred process, strontium carbonate and boric acid are used. The addition of boric acid is in the range of about 0.3 to 1.5 percent, by weight. The addition of a boron source at the start of the process has been found critical to achieving the magnetic properties hereinafter more fully described.

One of the principal advantages of our method is that it is not necessary that the raw iron oxide, specifically magnetite, be of high purity and small grain size as is required when using  $Fe_2O_3$ , but rather relatively low purity and large grained material is used. A suitable iron oxide for use in our process is "Meramac" iron oxide, a product of the Meramac Mining Company. "Meramac" is a technical grade iron oxide which analyzes at 93.02%  $Fe_3O_4$ , 6.15%  $Fe_2O_3$ , 0.1 percent silicon and 0.06 percent vanadium and less than 0.002 percent titanium, and which has a grain size on the order of 50 microns. "Meramac" currently is commercially available at a cost of 60-80 percent less than that of  $Fe_2O_3$  currently used in ferrite fabricating processes and, therefore, the use of "Meramac" significantly reduces the cost of fabricating hard ferrite magnets.

After weighing, the raw materials are then mixed with a sufficient amount of water and milled as a slurry in a stainless steel ball mill, block 12, for an extended period of time to achieve a thorough mixture of the raw materials. As a result of milling, the grain size of the magnetite is broken down from 50 microns to about 5 microns. The resulting mixture is then dried in an oven as shown by block 14. After drying, the material is screened into granules of a desired size, block 16, which are tumbled for a short time, block 18, to make the granules free-flowing. As a next step in the process, the material is fired or calcined at an elevated temperature wherein a reaction takes place to form the hexagonal ferrite, block 20. The ferrite material is mixed with water and comminuted, block 22, in a ball mill until ceramically workable particles of an average size of 1 to 2 microns are obtained. The ground ferrite, as a slurry, is then pressed in a non-magnetic die into a predetermined shape under a strong directional magnetic field, block 24, to remove the water and simultaneously

to orient the ferrite particles in the magnetic field. If desired, other methods of orienting and forming the ferrite crystals into a body may be used, such as dispersing the particles in a flexible, organic binder and mechanically orienting the particles therein to form a flexible sheet from which the magnetic bodies are cut. Such a method is described in U.S. Pat. No. 3,110,675 to Brailowsky owned by the assignee of this invention. The pressed body is then sintered in the temperature range of about 2,000° to 2,150° F, block 26, to form the finished magnet. The fired ferrite magnet may then be magnetized or, if desired, magnetization may be performed later.

The following specific examples will make the nature of our process and the resulting improved magnetic properties more clear.

#### EXAMPLE I

328.380 grams of "Meramac" iron oxide was mixed with 68.653 grams of strontium carbonate and 2.876 grams of boric acid to form a starting mixture having a composition of, by weight, 82.11 percent "Meramac", 17.17%  $SrCO_3$  and 0.72%  $H_3BO_3$ . The mixture was mixed and milled with water in a one-half gallon stainless steel ball mill for 14 hours, dried and screened through a 20 mesh screen. The granules were then tumbled for 15 minutes. Following tumbling, the mixture was calcined at 2150° F for 2 hours in a flowing air atmosphere. The calcined ferrite was then comminuted in water for 30 hours in a one-half gallon stainless steel ball mill having an equal number of  $\frac{3}{8}$  inch and  $\frac{1}{4}$  inch stainless steel balls. The comminuted particles as a slurry of about 45 to 48 percent, by weight, water were pressed in a directional magnetic field of 6,000 oersteds into cylindrical test samples one inch in diameter and one-half inch high. The density of the pressed samples was 2.75 g/cm<sup>3</sup>. The samples were then sintered in the range from 1900° to 2150° F for 30 minutes.

To demonstrate the effect of the boron addition, corresponding samples were prepared identically with the process described above, but without the boron addition. The intrinsic coercive force,  $H_{ci}$ , and remanence,  $B_r$ , of both sets of ferrite samples were then measured using a standard hysteresisgraph. Density measurements,  $D$ , were also made.

The tables below show the results of the hysteresisgraph measurements. The data shown below in Table I was obtained from the ferrite samples prepared in accordance with this invention, and the data shown in Table II was obtained from the identical samples, but prepared without the boron addition. The tabular data shown below in Table I is shown in graphical form in FIG. 2.

TABLE I

| Sintering Temperature °F | $H_{ci}$ OE | $B_r$ G | $D$ gr/cm <sup>3</sup> |
|--------------------------|-------------|---------|------------------------|
| 1900                     | 4,615       | 3,080   | 3.84                   |
| 1950                     | 4,385       | 3,435   | 4.22                   |
| 2000                     | 4,140       | 3,660   | 4.48                   |
| 2050                     | 4,105       | 3,740   | 4.65                   |
| 2100                     | 3,575       | 4,100   | 4.86                   |
| 2150                     | 3,280       | 4,040   | 4.98                   |

TABLE II

| Sintering Temperature °F | H <sub>c</sub> OE | B <sub>G</sub> | D gm/cm <sup>3</sup> |
|--------------------------|-------------------|----------------|----------------------|
| 1900                     | 4,425             | 2,485          | 3.16                 |
| 1950                     | 4,220             | 2,565          | 3.28                 |
| 2000                     | 3,765             | 2,845          | 3.60                 |
| 2050                     | 3,905             | 2,895          | 3.64                 |
| 2100                     | 2,275             | 3,725          | 4.49                 |
| 2150                     | 1,770             | 3,825          | 4.80                 |

Comparing the data in Table I with that in Table II it may be seen that in all respects the properties obtained in the ferrite samples prepared in accordance with this invention are superior to those prepared with magnetite and strontium carbonate, but without the boron addition. Further, from the data presented in Table I and from FIG. 2, it may be seen that the samples prepared in accordance with our improved process exhibited superior magnetic properties with a coincident numerical value of B<sub>G</sub> and H<sub>c</sub> at about 3,900 gauss and 3,900 oersteds, respectively, at a sintering temperature of about 2075° F (point A of FIG. 2). Although the samples prepared without the boron addition exhibited a relatively high intrinsic coercive force at the lower sintering temperatures and a relatively high remanence at the higher sintering temperature, the coincident numerical values of properties was only 3200 gauss and 3200 oersteds at a sintering temperature of about 2075° F.

Permanent magnets made in accordance with our process exhibit superior magnetic properties which are obtained at relatively low sintering temperatures. We have found that permanent magnets made in accordance with our process and sintered at about 2100° F are ideal for such applications as field magnets in dc motors since these magnets have a remanence of about 4100 gauss with a coercive force above 3500 oersteds.

Thus, a first feature of the invention is the use of coarse powder of natural magnetite together with boric acid as the additive.

A second feature of the invention is the timing of the boric acid introduction into the manufacturing process. We have found that it is very important to add the boric acid to the batch formula before the start of the first mixing, i.e., before the calcining operation. The introduction of the boric acid at this point results in a substantial improvement of the magnetic stability of the permanent magnets, i.e., in the improvement of the very "permanence" of the magnets which is measured by the value of the intrinsic coercive force. Such a feature of the invention can be of a decisive importance in fabrication of the ferrite magnets for applications such as the field magnets for dc motors. The following Example II demonstrates the effect of the timing on the magnetic stability as it is reflected by the intrinsic coercive force.

## EXAMPLE II

Two mixtures hereinafter referred to as Mixtures A and B were prepared using the same starting material and formula composition and the same manufacturing technique as in the Example I. The Mixtures A and B differ only in the timing of the boric acid introduction into the process. The boric acid was added to Mixture A before the first mixing, thus, before the calcining.

To the Mixture B the boric acid was added after the calcining, just before the grinding operation. With the exception of the calcining temperature and the grinding time which were in this Example 2100° F and 60 hours respectively, the process was identical to that of the Example I. The measuring technique was exactly as that as in the Example I. The results obtained are set forth in Tables III and IV.

TABLE III

| Sintering Temp. °F | Mixture "A"    |                   |                   |                                           |                       |
|--------------------|----------------|-------------------|-------------------|-------------------------------------------|-----------------------|
|                    | B <sub>G</sub> | H <sub>c</sub> OE | H <sub>c</sub> OE | (BH) <sub>max</sub> G-OE $\times 10^{-6}$ | D(g/cm <sup>3</sup> ) |
| 1950               | 3120           | 4360              | 2980              | 2.38                                      | 4.11                  |
| 2000               | 3250           | 4190              | 3050              | 2.69                                      | 4.41                  |
| 2050               | 3570           | 4030              | 3330              | 3.05                                      | 4.62                  |
| 2100               | 3780           | 3810              | 3540              | 3.36                                      | 4.79                  |
| 2150               | 3840           | 3570              | 3450              | 3.53                                      | 4.86                  |

TABLE IV

| Sintering Temp. °F | Mixture "B"    |                   |                   |                                           |                       |
|--------------------|----------------|-------------------|-------------------|-------------------------------------------|-----------------------|
|                    | B <sub>G</sub> | H <sub>c</sub> OE | H <sub>c</sub> OE | (BH) <sub>max</sub> G-OE $\times 10^{-6}$ | D(g/cm <sup>3</sup> ) |
| 1950               | 3110           | 3860              | 2930              | 1.97                                      | 4.28                  |
| 2000               | 3400           | 3780              | 3110              | 2.80                                      | 4.53                  |
| 2050               | 3570           | 3660              | 3280              | 3.00                                      | 4.77                  |
| 2100               | 3780           | 3500              | 3320              | 3.30                                      | 4.86                  |
| 2150               | 3830           | 3280              | 3110              | 3.52                                      | 4.95                  |

Examination of the Tables shows clearly that as compared with the addition of the boric acid after calcining, the addition of the boric acid before calcining results in a significant improvement of the magnetic stability of the ferrite magnets. Comparing the H<sub>c</sub> values of the Mixtures A and B it is apparent that the improvement takes place in the whole range of useful sintering temperatures.

Referring now to the demagnetizing curves shown in FIG. 3, it will be further seen that magnets made in accordance with our process have essentially straight line demagnetizing curves, which is ideal for dc motor applications. The two curves of FIG. 3, designated as curves I and II, are for two samples prepared according to our process and sintered at 2100° F for 30 and 15 minutes, respectively. The pertinent data for each sample is as follows:

Sample I

|                            |                    |
|----------------------------|--------------------|
| Sintering Temperature (°F) | 2100°              |
| Soak Time (min.)           | 30                 |
| B <sub>G</sub> (gauss)     | 4100               |
| H <sub>c</sub> (oersteds)  | 3500               |
| H <sub>c</sub> (oersteds)  | 3575               |
| (BH) <sub>max</sub> (gxoe) | 3.84 $\times 10^6$ |

Sample II

|                            |                    |
|----------------------------|--------------------|
| Sintering Temperature (°F) | 2100°              |
| Soak Time (min.)           | 15                 |
| B <sub>G</sub> (Gauss)     | 3900               |
| H <sub>c</sub> (oersteds)  | 3600               |
| H <sub>c</sub> (oersteds)  | 3825               |
| (BH) <sub>max</sub> (gxoe) | 3.53 $\times 10^6$ |

From the foregoing, it will be apparent that our improved process for making magnetically-anisotropic permanent magnets of the hard ferrite type yields magnets having superior properties which may be produced at a relatively low cost.

Although our invention has been described in terms of certain specific embodiments, it is to be understood that other forms may be adopted within the scope of our invention.

We claim:

1. A method of making a permanent magnet of the hard ferrite type having a hexagonal crystalline lattice with a magnetoplumbite structure and a formula  $\text{SrO} \cdot 6\text{Fe}_2\text{O}_3$ , comprising the steps of mixing and milling magnetite with a source of  $\text{SrO}$  and about 0.3 to 1.5 percent, by weight, of a compound selected from the group consisting of boric acid and boric oxide to form a homogeneous mixture thereof, calcining said mixture, comminuting said calcined mixture to form particles thereof having an average size of about 1 to 2 microns, compacting said particles while under the influence of a directional magnetic field into a body anisotropic in a principal direction, and sintering said body at a temperature in the range of 2000° to 2150° F.

2. The method of claim 1 wherein said mixture is calcined at about 2100° F.

3. A method of making a permanent magnet of the hard ferrite type having a hexagonal crystalline lattice with a magnetoplumbite structure and a formula  $\text{SrO} \cdot$

5  $6\text{Fe}_2\text{O}_3$ , comprising the steps of mixing and milling magnetite with a source of  $\text{SrO}$  and about 0.3 to 1.5 percent, by weight, of a compound selected from the group consisting of boric acid and boric oxide to form a homogeneous mixture thereof, calcining said mixture, comminuting said calcined mixture to form particles thereof having an average size of about 1 to 2 microns, compacting said particles while under the influence of a directional magnetic field into a body anisotropic in a principal direction, and sintering said body at a temperature in the range of 2000° to 2150° F.

10 4. A method of making a permanent magnet of the hard ferrite type having a hexagonal crystalline lattice with a magnetoplumbite structure and a formula  $\text{SrO} \cdot 6\text{Fe}_2\text{O}_3$ , comprising the steps of mixing and milling magnetite having an average grain size on the order of about 50 microns with a source of  $\text{SrO}$  and about 0.7 percent, by weight, boric acid to form a homogeneous mixture thereof, calcining said mixture of about 2100° F, comminuting said calcined mixture to form particles thereof having an average size of about 1 to 2 microns, compacting said particles while under the influence of a directional magnetic field to form a body anisotropic in a principal direction, and sintering said body in the range of 2000° to 2150° F.

15 20 25 5. The method of claim 4 wherein said body is sintered at about 2100° F.

\* \* \* \* \*